

## [54] CUTTING OIL COMPOSITION

[75] Inventor: Gifford George McClaflin, Ponca City, Okla.

[73] Assignee: Continental Oil Company, Ponca City, Okla.

[22] Filed: Mar. 8, 1973

[21] Appl. No.: 339,269

[52] U.S. Cl..... 252/46.7; 252/46.6; 252/56 R; 252/57

[51] Int. Cl.<sup>2</sup>..... C01M 1/48

[58] Field of Search..... 252/46.7, 46.6, 56 R, 57

## [56] References Cited

## UNITED STATES PATENTS

|           |         |                      |            |
|-----------|---------|----------------------|------------|
| 2,157,873 | 5/1939  | van Peski et al..... | 252/46.6   |
| 2,715,612 | 8/1955  | Beare.....           | 252/46.7 X |
| 2,734,868 | 2/1956  | Bright et al.....    | 252/46.7   |
| 2,830,024 | 4/1958  | Chapman et al.....   | 252/46.7   |
| 2,914,479 | 11/1959 | Tom et al.....       | 252/57 X   |
| 3,030,304 | 4/1962  | Elliott et al.....   | 252/46.7   |

|           |        |                   |            |
|-----------|--------|-------------------|------------|
| 3,071,549 | 1/1963 | Stark.....        | 252/57 X   |
| 3,208,945 | 9/1965 | Stuart et al..... | 252/57 X   |
| 3,273,981 | 9/1966 | Furey.....        | 252/56 R X |
| 3,492,232 | 1/1970 | Rosenberg.....    | 252/57 X   |
| 3,719,600 | 3/1973 | Bosniack.....     | 252/56 R X |

## OTHER PUBLICATIONS

Chemical Week, Oct.-Dec. 1971, (1972 Buyer's Guide in Act) Vol. 109, "Emery Organic Chemicals."

Primary Examiner—H. Sneed

Attorney, Agent, or Firm—Baylese E. Rutherford, Jr.

[57]

## ABSTRACT

A non-aqueous cutting oil composition is disclosed. The cutting oil composition comprises a major amount of paraffinic or naphthenic base oil and a minor amount of an additive combination which comprises: (a) sulfurized natural or synthetic sperm oil, (b) chlorinated paraffin, (c) trimer acid, and (d) dialkyl phosphite.

10 Claims, No Drawings

## CUTTING OIL COMPOSITION

## BACKGROUND

In metalworking operations, such as drilling, milling, sawing, threading, and the like, it is customary to use a liquid composition to carry away material removed in the operation and to prevent seizure of the metal to metal surfaces. In general, there are two types of cutting compositions, aqueous and non-aqueous. The present invention is concerned only with non-aqueous compositions. More specifically, the present invention is concerned with non-aqueous metalworking compositions having an additive combination which results in the final compositions having improved properties.

## PRIOR ART

A computer search of this art in broad terminology resulted in some 53 references, most of which were considered by the agent handling the case to be totally irrelevant.

The most pertinent references resulting from the computer search are believed to be the following U.S. Pat. Nos.: 2,612,477; 2,617,768; 2,698,304; 2,711,395; 2,890,172; 2,999,814; 3,017,352; 3,018,246; and 3,123,562.

The most pertinent art is believed to be the following:

The "Standard Handbook of Lubrication Engineering," McGraw-Hill, 1968, contains the following teachings:

1. it is known to use sulfurized sperm oil in cutting oils;
2. it is known to use chlorinated waxes and other chlorinated hydrocarbons as extreme pressure (E.P.) additives;
3. it is known to use organic phosphites as E.P. additives.

According to the "Chemical Week" 1972 Buyers' Guide Issue, dimer and trimer acids, available from Emery Industries, Inc., are suitable for use in metalworking lubricants.

The invention of the present application is believed patentable over the prior art for the following reasons. The specific additive combination gives improved E.P. properties. Use of a trimer acid gives better E.P. properties than does the dimer acid.

## BRIEF SUMMARY OF THE INVENTION

Broadly stated, the present invention is directed to a non-aqueous cutting oil composition comprising:

- a. a major amount of a paraffinic or naphthenic base oil, and
- b. a minor amount of an additive combination which comprises:
  - i. sulfurized sperm oil
  - ii. chlorinated paraffin
  - iii. trimer acid
  - iv. dialkyl phosphite

The specific amounts and nature of the materials used in the composition will be described in the detailed description.

## DETAILED DESCRIPTION

The base oil, which is used in a major amount of my composition, can be a paraffinic or naphthenic lubricating oil. Preferably, it is a naphthenic lubricating oil, and more preferably, it is a sulfurized naphthenic lubricating oil.

The term "naphthenic lubricating oil" is well known to those skilled in the art. Naphthenic oils have a greater amount of aromatics, lower viscosity indexes, and lower pour points than do the pale oils. The "sulfurized naphthenic oils" are naphthenic oils containing either natural and/or added sulfur. Usually, the amount of sulfur is in the range of 1 to 4 percent by weight. More usually, the amount of sulfur is from about 2 to about 3 percent by weight.

Suitable sperm oils include both natural and synthetic. The natural sperm oils are derived from the sperm whale and consist predominantly of monohydric fatty alcohol esters of fatty acids. Both the fatty alcohols and fatty acids are mixtures of saturated and unsaturated materials. The sperm oils are low in triglyceride content.

A complete description of sperm oils is found in the following book: "The Chemical Constitution of Natural Fats" by Hilditch and Williams, Fourth Edition, pp. 72 and 73 (book distributed in U.S. by Barnes & Noble, Inc.).

The synthetic sperm oils are materials which approximate the composition of the natural sperm oils. They are prepared by esterification of natural or synthetic fatty acids and fatty alcohols.

The sulfurized sperm oils (natural and synthetic) are prepared by reacting the original material with elemental sulfur or sulfur compounds to contain a specific amount of sulfur. The amount of sulfur is usually from 5 to 15 weight percent, more usually from 8 to 12 weight percent.

The term "chlorinated paraffin" is well known to those skilled in the art. Typically, it refers to materials having molecular weights in the range of from about 500 to about 600 and a chlorine content of about 30 to about 60, preferably about 40 to about 50, percent by weight.

The term "trimer acid" refers to aliphatic tricarboxylic acids produced by the polymerization of unsaturated fatty acids. Typically, they have acid values of 145-191 and saponification values of 170-210. Particularly suitable "trimer acids" are available from Emery Industries, Inc., under the trademark "Empol" 1040 and "Empol" 1041.

According to the 1972 Chemical Week Buyer's Guide "Empol" 1040 and "Empol" 1041 have the following typical composition:

|              | Dimer Acid <sup>(1)</sup> | Trimer Acid <sup>(2)</sup> |
|--------------|---------------------------|----------------------------|
| "Empol" 1040 | 20                        | 80                         |
| "Empol" 1041 | 10                        | 90                         |

<sup>(1)</sup>C<sub>20</sub> dibasic acid — M.W. Approx. 565

<sup>(2)</sup>C<sub>24</sub> tribasic acid — M.W. Approx. 845

Suitable dialkyl phosphites are those wherein the alkyl groups contain from about 10 to about 14 carbon atoms, preferably about 11 to about 13 carbon atoms. Dilauryl phosphite is particularly suitable.

The cutting oils of my invention contain the various additives in the following amounts:

|                      | PERCENT BY WEIGHT<br>Suitable | Preferred |
|----------------------|-------------------------------|-----------|
| Sulfurized Sperm Oil | 1-25                          | 2-10      |
| Chlorinated Paraffin | 0.5-10                        | 1-5       |
| Trimer Acid          | 0.25-5                        | 0.5-3     |
| Dialkyl Phosphite    | 0.1-5                         | 0.25-2    |

Of course, it is understood that the remainder of the composition comprises the base oil.

Use of a non-sulfurized base oil requires the use of larger amounts of sulfurized sperm oil, within the ranges stated above.

In order to illustrate the nature of the present invention still more clearly, the following examples, both illustrative and comparative, will be given. It is to be understood, however, that the invention is not to be limited to the specific conditions or details set forth in these examples except insofar as such limitations are specified in the appended claims.

The E.P. data were obtained using the Four-Ball test machine, as described in ASTM Method D-2783-69T, but using the conditions stated in the Examples. The Four-Ball machine and test method are also illustrated and described in a publication entitled "Lubrication Engineer's Manual" by National Tube Division of U.S. Steel Corp.

The materials used were the following:

#### Sulfurized Naphthenic Oil

A 50/50 blend of 100-115 SSU viscosity at 100°F and 150-160 SSU viscosity at 100°F. It has the following typical specifications: API gravity = 23-24; Natural sulfur = 1.5-1.7 wt percent;

Added sulfur = 0.85-1.0 wt percent.

#### Chlorinated Paraffin

Chlorine = 42 wt percent; Sp. Gr. = 1.185

Viscosity, SSU at 60°F = 9.87 — at 210°F = 170.

#### Trimer Acid

Containing 90 percent trimer acid and 10 percent

10

#### EXAMPLE 1

This example shows (1) that composition containing a combination of trimer acid and dilauryl phosphite is superior to compositions containing a combination of dimer acid and dilauryl phosphite, and (2) compositions containing the combination of trimer acid and dilauryl phosphite are superior to compositions containing no dilauryl phosphite.

15

| PERCENT BY WEIGHT<br>COMPOSITION NO. |      |      |      |
|--------------------------------------|------|------|------|
|                                      | A    | B    | C    |
| Sulfurized Naphthenic Oil            | 92.1 | 92.6 | 92.1 |
| Sulfurized Synthetic Sperm Oil       | 5.0  | 5.0  | 5.0  |
| Chlorinated Paraffin                 | 1.4  | 1.4  | 1.4  |
| Dimer Acid                           | 1.0  | —    | —    |
| Trimer Acid                          | —    | 1.0  | 1.0  |
| Dilauryl Phosphate                   | 0.5  | —    | 0.5  |

20

#### Four-Ball Test Results

| COMPOSITION NO.               |       |       |       |
|-------------------------------|-------|-------|-------|
|                               | A     | B     | C     |
| Weld, Kg <sup>(1)</sup>       | 420   | 500+  | 500+  |
| No-Seizure, Kg <sup>(1)</sup> | 50    | 55    | 65    |
| Wear <sup>(2)</sup>           | 0.330 | 0.485 | 0.327 |

<sup>(1)</sup>Weld and No-Seizure at 10 seconds and 1800 RPM.

<sup>(2)</sup>Wear-one hour, 1800 RPM, 20 Kg.

25

#### EXAMPLE 2

This example shows that Composition C of Example 1 is superior to three commercial cutting oils in that the maximum no-seizure load decreases with increasing temperature for the commercial cutting oils but not for Composition C.

30

#### Four-Ball Maximum No-Seizure Load, Kg (10 Seconds at 1800 RPM)

| Composition        | TEMPERATURE |       |       |       |       |
|--------------------|-------------|-------|-------|-------|-------|
|                    | Ambient     | 150°F | 250°F | 350°F | 400°F |
| C from Ex. 1       | 65          | —     | 75    | —     | 65    |
| Commercial Oil "X" | 72          | 72    | 46    | 16    | 10    |
| Commercial Oil "Y" | 63          | 53    | 50    | 13    | 7     |
| Commercial Oil "Z" | 57          | 55    | 43    | 4     | 3     |

35

#### EXAMPLE 3

This example shows that sulfurized sperm oil can be substituted for sulfurized synthetic sperm oil.

40

|                                | COMPOSITION NO.      |    |
|--------------------------------|----------------------|----|
|                                | PERCENT BY<br>WEIGHT |    |
|                                | D                    | E  |
| Sulfurized Naphthenic Oil      | 97                   | 95 |
| Sulfurized Sperm Oil           | 3                    | —  |
| Sulfurized Synthetic Sperm Oil | —                    | 5  |

45

#### Four-Ball Results Weld, Kg, 10 Seconds, 1800 RPM

| Composition No. | D    | E    |
|-----------------|------|------|
| Weld, Kg        | 400+ | 400+ |

50

Thus, having described the invention in detail, it will be understood by those skilled in the art that certain variations and modifications may be made without de-

#### Sulfurized Synthetic Sperm Oil

Sulfur = 10.0 weight percent; Active sulfur = none; Saponification number = 212; Viscosity at 210°F = 158 SSU.

#### Sulfurized Sperm Oil

Sulfur = 10.0 weight percent; Viscosity at 210°F = 200 SSU.

parting from the spirit and scope of the invention as defined herein and in the appended claims.

I claim:

1. A non-aqueous cutting oil composition comprising (a) from about 55 to about 98 weight percent of a paraffinic or naphthenic base oil and (b) the combination of the following materials in the amounts specified:

| Percent by Weight    |                       |
|----------------------|-----------------------|
| Sulfurized Sperm Oil | About 1 to about 25   |
| Chlorinated Paraffin | About 0.5 to about 10 |
| Trimer Acid          | About 0.25 to about 5 |
| Dialkyl Phosphite    | About 0.1 to about 5  |

said composition being characterized further in that

- a. said sulfurized sperm oil contains about 5 to about 15 weight percent sulfur,
- b. said chlorinated paraffin contains about 30 to about 60 weight percent chlorine, and
- c. said trimer acid contains at least 80 percent C<sub>54</sub> tri-basic acids.

2. The composition of claim 1 wherein the base oil is a sulfurized naphthenic lubricating oil.

3. The composition of claim 2 wherein the dialkyl phosphite is dilauryl phosphite.

4. A non-aqueous cutting oil composition comprising from about 80 to about 96 weight percent of a paraffinic or naphthenic base oil and the combination of the following materials in the amounts specified:

| Percent by Weight    |                       |
|----------------------|-----------------------|
| Sulfurized Sperm Oil | About 2 to about 10   |
| Chlorinated Paraffin | About 1 to about 5    |
| Trimer Acid          | About 0.5 to about 3  |
| Dialkyl Phosphite    | About 0.25 to about 2 |

said composition being characterized further in that

- a. said sulfurized sperm oil contains about 5 to about 15 weight percent sulfur,

10

- b. said chlorinated paraffin contains about 30 to about 60 weight percent chlorine, and
- c. said trimer acid contains at least 80 percent C<sub>54</sub> tri-basic acids.

5 5. The composition of claim 4 wherein the base oil is a sulfurized naphthenic lubricating oil.

6. The composition of claim 5 wherein the dialkyl phosphite is dilauryl phosphite.

7. The composition of claim 6 wherein:

- a. the sulfurized naphthenic base oil contains about 1 to about 4 percent by weight sulfur,
- b. the chlorinated paraffin has a molecular weight in the range of about 500 to about 600, and
- c. the trimer acid has an acid value of about 145 to about 191 and a saponification number of about 170 to 210.

8. The composition of claim 7 wherein:

- a. the sulfurized naphthenic base oil contains about 2 to about 3 weight percent sulfur,
- b. the chlorinated paraffin contains about 40 to about 50 weight percent chlorine, and
- c. the sulfurized sperm oil contains about 8 to about 12 weight percent sulfur.

9. The composition of claim 8 wherein the sulfurized sperm oil is a synthetic sperm oil.

10. The composition of claim 9 wherein the specified materials are present in the following amounts:

25

| Percent by Weight              |           |
|--------------------------------|-----------|
| Sulfurized Synthetic Sperm Oil | About 5   |
| Chlorinated Paraffin           | About 1.4 |
| Trimer Acid                    | About 1   |
| Dilauryl Phosphite             | About 0.5 |

\* \* \* \* \*

30

35

40

45

50

55

60

65